

(No Model.)

J. H. CARPENTER.

PROCESS OF MANUFACTURING COLORED PAPER.

No. 443,658.

Patented Dec. 30, 1890.



FIG II



WITNESSES:

Rodmond K. Beach  
Francis G. Beach

INVENTOR

James H. Carpenter  
BY  
John K. Beach

ATTORNEY

# UNITED STATES PATENT OFFICE.

JAMES H. CARPENTER, OF CHICAGO, ILLINOIS, ASSIGNOR OF TWO-THIRDS TO CHARLES E. O'HARA, OF NEW YORK, N. Y., AND THE SEYMOUR PAPER COMPANY, OF WINDSOR LOCKS, CONNECTICUT.

## PROCESS OF MANUFACTURING COLORED PAPER.

SPECIFICATION forming part of Letters Patent No. 443,658, dated December 30, 1890.

Application filed March 31, 1890. Serial No. 346,089. (No specimens.)

*To all whom it may concern.*

Be it known that I, JAMES H. CARPENTER, a citizen of the United States, residing at Chicago, in the county of Cook and State of Illinois, have invented a new and useful Process 5 of Manufacturing Colored Paper, of which the following is a specification.

In my process the pulp is first prepared for paper-making in the usual way by agitation 10 with water. The coloring-matter is then irregularly mixed with the pulp while the pulp is in such relation to the web-forming devices that the diffusion of color may be checked by the immediate withdrawal of the water from 15 the pulp in the process of forming the web before a uniform tint is reached and then pressing and drying the web in the usual way. By this process shaded and clouded color effects are produced in the finished paper.

20 In the drawings, Figure 1 represents a portion of the "Fourdrinier machine," so called, in which B B B are the suction-boxes; D, the dandy-roll; C, the couch-rolls, and F a tube conveying coloring-matter to the pulp at or 25 near the point A.

In Fig. 2, which represents a portion of a "cylinder-machine," so-called, G is the vat, II the cylinder, and F a tube conveying coloring-matter to the pulp at or near the point A.

30 The drawings show only so much of the machines, respectively, as is necessary to illustrate the application of my new process thereto.

It is essential that the coloring-matter 35 should be irregularly mixed with the pulp while it is in a fluid or semi-fluid state and before it has been formed into a web. Otherwise unsightly strips and blotches of color are produced, having abrupt and ragged edges, 40 because no sufficient diffusion of the color takes place to soften and shade the edges of the color-patches. It is also essential that the withdrawal of the water from the pulp should begin immediately after the introduction 45 of the coloring material. Otherwise the color will spread and diffuse itself throughout the pulp, so as to produce a uniform tint in the finished paper.

My process is especially well adapted to be

used in the manufacture of colored paper on 50 machines of the types known as the "Fourdrinier" and "cylinder" machines, and I have found that the most favorable results are obtained when the color is applied at or near the "sluices" on the Fourdrinier machine 55 and at or just beneath the surface of the fluid pulp in the cylinder-machine.

In the Fourdrinier machine the pulp or stuff suspended in water is fed, as is well known, to a horizontally-moving endless apron of fine 60 wire-cloth, called the "Fourdrinier" or "making" wire, which carries the layer of pulp along and at the same time is shaken laterally to facilitate the interlocking or felting of the fibers, and during this operation the water is drained off through the meshes of the wire, first by gravity and afterward by suction-boxes, until the pulp, which at the beginning of its journey was a mass of freely-moving fibers suspended in water, has taken 70 on the consistency of a web of wet pulp when it is delivered from the making-wire to a felt apron to be pressed, dried, and finished into paper.

When the Fourdrinier machine is used, the 75 color, which may consist of an aqueous solution of aniline dye, (though I do not limit myself thereto,) should be applied in a stream or shower to the pulp at or near the point where it enters on the making-wire, as shown 80 at Fig. 1, A being the point at which the pulp is fed to the making-wire.

In the cylinder-machine the general mode of operation is the same, the making-wire being in the form of a cylinder partially submerged in the pulp instead of a horizontally-moving web. In this machine the water holding the pulp in suspension escapes through the meshes of the submerged part of the cylinder, leaving a layer of pulp adhering thereto, which is lifted out of the vat by the rotation of the cylinder. When the cylinder-machine is used, the color should be added to the pulp in the vat at a point adjacent to the cylinder and upon or just below the surface 95 of the pulp, so that the coloring-matter will be drawn toward the cylinder by the current of escaping water and will not be diffused

generally throughout the vat. The proper point for applying the color in this class of machines is illustrated in Fig. 2.

When two or more streams or showers of coloring-matter are used, the colors or tints are shaded and blended together according as the points of application are more or less widely separated, and by varying the relative position of the points of application and the amount and character of the coloring-matter an endless variety of artistic effects may be produced. In spite of this variety the product is always characterized by a peculiar softness of shading or clouding of the tints, and can be readily distinguished from colored paper made in the ordinary way or from paper printed in colors or tints.

What I claim, and desire to secure by Letters Patent, is—

The process of manufacturing paper colored in clouded and shaded tints, which consists in preparing the pulp for paper-making by agitation with water in the usual way, mixing coloring-matter irregularly with the pulp, immediately withdrawing the water in the process of forming the web before a uniform tint has been imparted to the web, and then pressing and drying the colored web in the usual way, substantially as and for the purpose described.

JAMES H. CARPENTER.

Witnesses:

ROBT. I. HUNT,  
HENRY C. MURCH.